

Jan. 12, 1932.

A. E. HALL

1,840,946

LEAD REFINING APPARATUS

Filed Nov. 8, 1929

3 Sheets-Sheet 1



Jan. 12, 1932.

A. E. HALL

1,840,946

LEAD REFINING APPARATUS

Filed Nov. 8, 1929

3 Sheets-Sheet 2



Fig. 4.

INVENTOR

Arthur E. Hall

BY

MacCloskey & Neal  
ATTORNEYS

Jan. 12, 1932.

A. E. HALL

1,840,946

LEAD REFINING APPARATUS

Filed Nov. 8, 1929

3 Sheets-Sheet 3



Fig. 5.



Fig. 6.

INVENTOR  
Arthur E. Hall  
BY  
Harr Cross & Neal  
ATTORNEYS

## UNITED STATES PATENT OFFICE

ARTHUR E. HALL, OF PERTH AMBOY, NEW JERSEY

## LEAD REFINING APPARATUS

Application filed November 8, 1929. Serial No. 405,573.

This invention relates to lead refining and is more particularly directed to a process and apparatus for the removal of bismuth from lead.

The metal bismuth is found as an impurity in lead and when present in even small quantities, say upwards of 0.15%, renders the lead unsatisfactory to a large portion of the lead consumers. Cable sheathing, lead pipe, sheet lead, battery plate grids and lead for paint making purposes and other purposes will not tolerate lead containing even small quantities such as 0.15%. If the bismuth content is reduced to 0.034% or less the lead produced is satisfactory to the trade. At the present time it is possible to produce lead containing such low quantities of bismuth by the electrolytic process of refining, and by segregating ores, but the electrolytic process is an expensive one and its expense increases as the quantity of bismuth in the lead increases. Where lead bismuth contains less than approximately 97% lead it has been found advisable to apply both a fire process and later an electrolytic process on the same lead with the combined cost of a little less than 1¢ per pound for such treatments.

In 1900 Stephen Tredinnick who had been working at a plant in Nevada where the separation of silver from lead was being practiced, was granted a U. S. Patent No. 662,836 for an apparatus for refining and desilverizing lead, and somewhat later it was attempted to employ the apparatus described in his patent for the removal of bismuth from lead and the concentration of the bismuth in a relatively small amount of lead. The apparatus involved included a number of kettles which were separately heated and agitated in an attempt to insure uniform heating throughout by blowing steam into the kettles. After heating up of a charge in one kettle, it was allowed to crystallize in part and the kettle was then lifted by a hydraulic ram and the molten contents were allowed to flow into a second and adjacent kettle, after which the remaining crystals were melted in the first kettle and then, this kettle still being elevated by means of the hydraulic ram, the melted crystals were transferred by gravity to a third

and adjacent kettle. The process was not a continuous one and involved a large percentage of idle equipment containing metallic lead whose processing was awaiting the release of other apparatus in the refining group. The apparatus also presented considerable other difficulties in operation which resulted in a relatively small output and an exorbitant cost along with poisoning of the operatives due to the production of fine particles of dross blown up by the steam used in agitation of the kettles. These disadvantages resulted in abandonment of the Tredinnick apparatus for the purpose mentioned and since then it has been necessary to rely on the costly and laborious electrolytic process.

The principal object of this invention accordingly is to provide a simple, inexpensive, and efficient apparatus for refining lead to lower its bismuth content which shall do away with the disadvantages of the electrolytic process and practice mentioned under the Tredinnick patent. Another object of the invention is to provide a simple efficient apparatus which shall permit a continuous separation of bismuth from lead, which shall avoid holding large masses of lead idle while waiting for available apparatus for processing, which shall permit a simple effective control to be maintained for the production of lead containing desired percentages of bismuth and in accordance with the bismuth content of the raw material as received. Other objects will be in part obvious and in part pointed out hereinafter.

The invention accordingly comprises the novel apparatus and combinations thereof, specific embodiments of which are described herein by way of example only and in accordance with the manner in which I now prefer to practice the invention.

Further and more specific objects, features and advantages will clearly appear from the detailed description given below taken in connection with the accompanying drawings which form a part of this specification and illustrate by way of example one embodiment of the invention.

In the drawings, Fig. 1 is a diagrammatic plan view of a preferred embodiment of my

invention, the driving shafts for crystal conveyors and certain other parts being omitted for the sake of clearness;

Fig. 2 is a corresponding diagrammatic elevation of a preferred embodiment of my invention;

Fig. 3 is a detail sectional elevation taken on the line 3—3 of Fig. 1 showing the crystallizer with a spiral conveyor and its driving means moving lead bismuth crystals out of the molten lead containing a higher content of bismuth, these crystals being deposited in a heated kettle on the right;

Fig. 4 is a diagrammatic end elevation of the series of crystallizers and kettles;

Fig. 5 is a sectional plan view of a part of the series of crystallizers and kettles taken on the line 5—5 of Fig. 3, certain parts being omitted for the sake of clearness; and

Fig. 6 is a sectional elevation taken on the line 6—6 of Fig. 5.

Referring now to the drawings, and particularly to Figs. 1 and 2, I have designated a series of crystallizers or baths there shown as C1 to C13 inclusive and the kettles corresponding thereto and into which each crystallizer or bath delivers to K1 to K13 respectively and inclusive. These crystallizers and kettle units constitute a series at one end of which, namely at K1, lead of the lowest bismuth content produced is obtained and at the opposite end of the series lead with the highest bismuth content is obtained.

These crystallizer-kettle units, C1, K1, C2, K2, C3, K3 and so on are positioned so as to maintain therethrough a continuous and unobstructed gravity flow of lead-bismuth in which the bismuth is increasing and an opposite flow which is partially by gravity of lead-bismuth with increasing content of lead. To accomplish the gravity flow, each crystallizer, for example C1, is set at a height, preferably 6 inches above the next crystallizer C2 in the series. In accordance with this arrangement, the metal level of C2 is at a height of 6 inches higher than the metal level of C3, and the metal level of C3 is at a height of 6 inches higher than the metal level of C4, and so on through the series. Between each crystallizer or bath is a substantially horizontal open launder serving to convey molten lead-bismuth alloy from one crystallizer or bath to the next by gravity due to the head existing between the crystallizers, thus between C1 and C2 is a launder L1, between C2 and C3 is a launder L2 and so on throughout the series of launders L3 to L12 occur, L12 being positioned between crystallizer C12 and C13 and a launder L13 serving as an exit for the lead containing higher bismuth.

The flow of lead-bismuth alloy in which the amount of lead is increasing is maintained by continuously rotating screws and partially

by gravity. Each of the crystallizers is provided with respective screws S1 to S13. These screws are of a particular construction which will be described hereinafter. The crystallizers or baths are maintained at a suitable temperature to keep a molten mass of combined lead and bismuth with crystals of lead-bismuth, which crystals will naturally contain less bismuth than the bismuth content of the molten mass, and correspondingly more lead. The proportion of lead-bismuth crystals to molten metal in the baths will be maintained at a ratio which will give desired results. I find 57% crystals and 43% molten metal maintains proper grades in the case where the raw material containing 0.164% bismuth is charged into K6 when a product from K1 is desired containing 0.034% bismuth, but other grades of raw material and other desired grades of products may indicate other proportions.

The crystals are moved out of the crystallizer or bath by the rotating screws, each screw delivering into its corresponding kettle at a pre-determined rate depending upon the area of the screw and of course upon the proportion of crystals to molten metal present as determined by the temperature maintained. In each kettle the crystals received are melted by an oil burner or other source of heat and in melted condition are allowed to flow by gravity through a series of open ducts or launders D1 to D12 inclusive. The duct leading from the kettle K2 to crystallizer C1 is designated as D1, from the kettle K3 to C2 is designated as D2 and so on to the end of the series. The duct D13 leads from the kettle K1 and is an outlet for the lead containing the lowest content of bismuth. The launders L1 to L12 inclusive and the ducts D1 to D12 inclusive are so positioned that the hot gases issuing from the combustion chambers of the respective oil burners under the respective kettles in part or in whole surround the launders and ducts to prevent chills and stoppages in same.

A typical crystallizer and kettle construction is shown in Fig. 3. The crystallizer and kettle there shown are those designated in Figs. 1 and 2 as C6 and K6. The crystallizer is in the form of an open trough of suitable material such as cast iron mounted in a base 1 of concrete or other suitable material. The bottom 2 of the crystallizer is inclined at an angle of about 90° to the lower end wall 3 of the crystallizer and the bottom wall is set at about an angle of 40° to the horizontal being held in position by the concrete base 1. Mounted in suitable bearings on the end walls is a rotatable shaft 4 which is rotated by an outside source of power not shown, which outside source of power rotates corresponding shafts to which each of the respective screws S1 to S13 are attached. The screw S6 there shown is attached to shaft 4

and is in the form of a helix being perforated throughout with drawing holes 5 about  $\frac{1}{16}$  inches, preferably, in diameter. The bath of lead-bismuth 6 contains approximately the ratio 57% crystals to 43% molten mass and the screw 6 as it rotates moves these crystals out of the molten bath, draining back any molten material through the perforations 5, the crystals being deposited in the kettle K6. The kettle K6 is mounted on suitable pillars of refractory material 7 and is surrounded by a refractory fire wall 8 through which an oil burner 9 for supplying heat to the kettle K6 is provided. The crystals passing into the kettle K6 are melted there and then flow back through the duct D5 into the crystallizer C5. The temperature of the molten crystals in K6 is maintained so that when these crystals reach C5 they will be at the proper temperature to maintain a ratio of crystals to molten material of the desired 57% crystals to 43% molten material or any desired proportion. This temperature is maintained by suitable regulation of the heat provided by the oil burner 9.

The arrangement for heating the upper portion of the crystallizers is shown in Figs. 5 and 6. The description of one heating means for a crystallizer will suffice for all as the heating means is preferably identical throughout. As shown in Figs. 5 and 6, the gases passing from the burner 9 pass under the kettle K6 and up through two ducts 10 and 11 at the end of the kettle on either side of the crystallizer. These ducts are controlled by hand-operated dampers 12 and 13 to allow part or all of the gas to pass upwardly without passing around the crystallizer C6 or else part or substantially all of the burner gases may pass along the side walls of the crystallizer in order to heat that part of the crystallizer above the level of the lead therein. For this purpose openings 14 and 15 are provided respectively in the ducts 10 and 11 at a point between the lead level in crystallizer C6 and the top of the crystallizer tank. This duct leads respectively into flues 16 and 17, each of which is shaped to follow the outline of the crystallizer wall above the lead level. At the end of the crystallizer away from the ducts 10 and 11 the flues 16 and 17 are flattened out as shown in Fig. 5 joining one another to make a flattened flue 18 which communicates by a branch 19 with a common pipe 20 leading to the stack 21. Gases from flues 10 and 11 after passing therethrough may also be led to the stack 21 by connections not shown.

Dampers 12 and 13 are provided with handles so that they may be moved in the ducts 10 and 11 and positioned to cause all of the gases to pass up the conduits 10 and 11 when it is not desired to heat the upper part of the crystallizers or to divert part or all of the gases along the flues 16 and 17 to

heat the upper part of the crystallizers desired.

Each of the flues 16 and 17 has a crystallizer wall forming one vertical side of it in each case, the other walls of the flues as well as the walls of the ducts being made of suitable refractory material. These heated flues serve the purpose of preventing solid chills on the inner side of the wall above the molten metal level thereof. Such chills are to be avoided because they not only impede the rotary movement of the screws but cause a solid lead bismuth compound to form which may be different from the constitution of the crystals in the crystallizers.

Each of the screw conveyors S1 to S13 is driven in a manner similar to that shown with the screw conveyor S6 in Fig. 3. A common shaft 22 drives the various screw conveyors. A tooth pulley 23 is mounted opposite each crystallizer tank communicating through a chain 24 with tooth pulley 25 mounted to drive a worm 27 mounted on the crystallizer and driving a worm wheel 28. The latter is mounted on the end of the shaft 4 of the screw conveyor S6. I preferably maintain the revolutions per minute of all screw conveyors the same. Once started the speed of these conveyors need not be adjusted. The rate of crystal delivery into the kettles is controlled as heretofore pointed out by the temperature maintained in the crystallizers and hence the quantity of crystals produced. This temperature is adjusted by means of the oil burners underneath the various kettles and control of the plant by control of the heat supplied to these burners so that a greater or less tonnage to be produced at the ends of the series is secured.

The typical crystallizer and kettle shown in Fig. 3 is repeated in each of the other crystallizers and kettles represented in the group C1 to C13 inclusive and K1 to K13 inclusive, including the inclination of the crystallizer, the form of the conveyor, positioning of the kettle and the oil burner, ducts and flues for adjusting the temperature thereof.

As shown particularly in Figs. 1 and 2, the respective diameters and areas of the kettles, crystallizers and screws varies, the larger ones being on the left and being graduated to the smallest on the right of the series. This graduation is arranged proportionately to the amount of work done by each unit.

The overflow levels for the various crystallizers for crystals being moved into the respective kettles are designated respectively as O1 to O13 inclusive, see particularly Fig. 4.

In carrying out the process of separating lead from bismuth, lead containing bismuth in the proportion of .164% as an example, is available as a starting material and is employed in the process although it will be understood that lead with higher or lower bis-

muth contents may be employed to commence the process. This material is melted and charged into the crystallizer C6 where it attains a temperature such that the mass will contain approximately 57% of lead-bismuth with crystals and about 43% of molten material approximately 317° to 327° C. The screw conveyors S1 to S13 are started to rotate and the oil burners for kettles K1 to K13 are started to bring the temperatures in these various kettles up to the proper points, all of the crystallizers having been brought to and being maintained at a suitable temperature for providing the desired ratio of crystals to molten material therein as received. The crystals are continuously transferred from the crystallizer into the melting kettle K6 which is now at a suitable temperature to melt the crystals whereupon they flow through D5 into crystallizer C5 which is at a suitable temperature to maintain the ratio of crystal to molten condition of 57% to 43% or any desired ratio. The screw conveyor there removes these crystals as they form and moves them into the kettle K5 where they are melted. The molten material in C5 due to the position of C5 above C6 tends to flow and in part flows through L5 back into C6 where it joins molten material already there. C6 is maintained by the molten metal flowing from K7 and also by the heated gases from the combustion chamber of K6 at a slightly lower temperature than C5 where temperature is maintained by inflowing molten metal from K6 and also by regulated diversion of heated gases from combustion chamber of K5 so that from the molten material flowing from C5 to C6 through L5 some crystals form and these join crystals forming from molten material already present in C6 and these combined crystals are moved as indicated by S6 into the kettle K6. C6 is supplied, of course, it will be understood by fresh lots of the raw material containing bismuth of approximately .164%. The molten material in C6 will tend to flow from it to C7 due to the height of C6 above C7. C7 is maintained at slightly lower temperature than C6 and crystals form therein, these crystals being removed from S7 into K7. In K7 a similar process to that occurring in K6 results and K7 being 6 inches higher than C6 the melted crystals flow back into C6. The molten material in C7 passes through L7 into C8. The crystals of lead-bismuth containing a higher content of lead are those flowing by combined screw action and gravity in a direction towards K1 from which the material lowest in bismuth and highest in lead is obtained. The lead containing bismuth is fed in molten condition from a tank T which may be connected to any one of the intermediate kettles. In this case it is shown as connected to K6 (see Fig. 1) and is intended to supply as there connected, lead containing preferably

a bismuth content of about 0.164%. If lead with a lower bismuth content were supplied this tank could be connected to kettle K4, K3, or if lead with a higher bismuth content were supplied the tank could be connected to K7, K8, etc. Tank T is connected to kettle K6 by means of a pipe in which is connected a centrifugal pump which is intended to continuously feed the molten raw material at a temperature slightly above its melting point into the crystallizer. As shown on Fig. 1, the successive degrees of the average bismuth content of the whole mass in each crystallizer or bath from C13 to C1 are 1.46%, 1.00%, .784%, .572%, .418%, .308%, .224%, .164%, .12%, .091%, .067%, .05%, .042%.  
70  
75

The molten material is flowing entirely by gravity as I prefer from C1 to C2, from C2 to C3 and so on through the series, C1 to C13 having successive degrees in bismuth content of .05% to 2.00% in the same stages just mentioned but in the reverse direction.  
85

On the other hand the molten material is flowing entirely by gravity as I prefer, through the series K13 to C12, K12 to C11, and so on from K13 to K1 to final product issuing from K1 of a grade of 0.034% bismuth, according to the stages first mentioned. The crystals collected in K1 therefore will have a bismuth content of approximately 0.034% or less and a lead content of approximately 99.9%+.  
90  
95

On the other hand the molten material containing the higher contents of bismuth is flowing entirely by gravity, as I prefer, through the series of kettles from K1 to K13 with a bismuth content increasing from .042% to 1.460% bismuth, according to the stages just mentioned, in the reverse direction.  
100  
105

It will be understood that although I have shown and described in the specification the production of a lead containing 2.00% of bismuth, the content of bismuth in the product passing from C13 may range to higher percentages of bismuth towards that alloy of lead and bismuth which has the lowest melting point and contains a higher percentage of bismuth.  
110

The apparatus and process mentioned are simple and efficient. The rate of flow is all controlled automatically, there are no troublesome valves to get out of order requiring manual manipulation, the only control being exercised by proper regulation of the temperature provided by the oil burners, which in turn controls the relative percentage of crystals and liquid in the crystallizers and hence the delivery of crystals from the crystallizers to the kettles. The separation of crystals from molten material by the perforated screw conveyors is clean and effective and the melting of the crystals introduced into the kettles is efficiently performed because a relatively small mass of unmelted  
115  
120  
125  
130

material is dropped into a large mass of molten material. The provision of a 6 inch head of molten metal throughout the system insures that no great pressure of this material will be exerted on the connections between the various pieces of apparatus so that a long life is assured to them and to the apparatus. In case it is necessary to make replacements, however, these may be made promptly and inexpensively. In addition capital outlay for the building of such a plant is relatively small. The apparatus is so arranged in addition that there is no violent agitation or large exposure of molten metal surface and hence a minimum oxidation of lead occurs with minimum presence of fume and danger of poisoning of the operatives is thus avoided.

The process is continuous and eliminates delay in the units. There is no mass of molten material waiting for a kettle or crystallizer to be free before it can be processed. After the temperatures have been adjusted throughout the units the process can be operated without change of temperature in the units as long as the raw material being supplied is of approximately the same bismuth content and it is desired to produce a lead of approximately the same lowered bismuth content. One advantage resulting from the maintenance of a uniform temperature is that it is not necessary to cool down or heat up large masses of refractory material which are naturally poor conductors radiators and absorbers of heat. The process is applicable of course to lead materials with varying bismuth contents and in accordance with the temperature control, the poundage or tonnage, issuing from either the low bismuth end or the high bismuth end may be adjusted. The desired flow of metal, namely lead concentrate in one direction and bismuth concentrate in the opposite direction is automatically obtained by reason of the established levels of the crystallizers and kettles and flow in any other direction is prevented.

While I have described my invention in considerable detail and with respect to a preferred form thereof, I do not desire to be limited to such details or form since many changes and modifications may be made and the invention embodied in widely different forms without departing from the spirit and scope thereof in its broader aspects. Therefore, I desire to cover all modifications and forms coming within the language or scope of any one or more of the appended claims.

What I claim as new and desire to secure by Letters Patent is:

1. In apparatus for refining lead, in combination, a kettle and a crystallizer, automatic means for continuously moving crystals out of the crystallizer into the kettle, means for melting said crystals in the kettle and delivering them in molten condition out-

side of said kettle, and means to conduct molten material away from the crystallizer.

2. In apparatus for refining lead, in combination, a crystallizer-kettle unit having a kettle and crystallizer, means for moving crystals out of the crystallizer into the kettle, means for melting said crystals in the kettle and delivering them in molten condition to another crystallizer-kettle unit, and means to conduct the molten material away from the crystallizer to a third unit.

3. In apparatus for refining lead, in combination, a crystallizer-kettle unit having a kettle and crystallizer, means for moving crystals out of the crystallizer into the kettle, means for melting said crystals in the kettle and delivering them in molten condition to the crystallizer of another crystallizer-kettle unit and means to conduct molten material away from the first mentioned crystallizer to the crystallizer of a third crystallizer-kettle unit.

4. In apparatus for refining lead, in combination, a series of crystallizer-kettle units arranged in a sequence to provide an unobstructed gravity flow of molten lead containing an increasing amount of impurities such as bismuth in one direction, and providing a flow of lead containing decreasing amounts of impurities such as bismuth in an opposite direction, each unit having a kettle and a crystallizer, means for moving crystals out of the crystallizer into the kettle, means for melting said crystals in the kettle and delivering them in molten condition outside of said unit, and means to conduct molten material away from the crystallizer.

5. In apparatus for refining lead, in combination, a series of crystallizer-kettle units arranged in a sequence to provide an unobstructed gravity flow of molten lead containing impurities such as bismuth in one direction, and providing a flow of lead containing decreasing amounts of impurities such as bismuth in an opposite direction, each unit having a kettle and a crystallizer, a conveyor in each crystallizer for conveying crystals out of it into the kettle, a heater for melting crystals in the kettle, a duct connecting said kettle with the next crystallizer on one side of the series and being positioned to allow a gravity flow of molten material from the kettle to said other crystallizer and a duct for conducting molten material away from the crystallizer to the next crystallizer on the other side of the series.

6. In apparatus for refining lead, in combination, a series of crystallizer-kettle units arranged in a sequence to provide an unobstructed gravity flow of molten lead containing an increasing amount of impurities such as bismuth in one direction; and providing a flow of lead containing decreasing amounts of impurities such as bismuth in an opposite direction, each unit having a kettle, a crystal-

- lizer and a conveyor for moving crystals out of the crystallizer into the kettle and a heater for heating crystals in the kettle, each of the crystallizer-kettle units being connected to the units on either side thereof except at the end of the series by a duct leading from the kettle to the crystallizer of the unit on one side for delivering melted crystals by gravity from the kettle to said crystallizer, and a launder leading from the last mentioned crystallizer to the first mentioned crystallizer for delivering molten lead containing increasing impurity, by gravity, to the first mentioned crystallizer, the crystallizer-kettle unit on the other side having a duct leading from its kettle to the first mentioned crystallizer and delivering melted crystals containing increasing lead content by gravity to the crystallizer, and a launder leading from the first mentioned crystallizer to the crystallizer of the last mentioned unit to deliver molten lead containing increasing impurity by gravity to the crystallizer of the last mentioned unit, the crystallizer-kettle units at either end being connected in a similar manner to that described on the other units but being connected to deliver, respectively, outside the series for molding or otherwise, material of the highest lead content and material of the lowest lead content.
7. In apparatus for refining lead, in combination, a series of crystallizers and kettles, arranged in a sequence to provide a flow of molten lead containing an increasing amount of impurities such as bismuth in one direction and providing a flow of lead containing decreasing amounts of bismuth in an opposite direction, each crystallizer having a conveyor for moving crystals out of the crystallizer into the kettle, connections between the kettles and crystallizers in the series, the dimensions of the crystallizers, kettles and conveyors being proportioned to the amounts of material to be handled by each.
8. In apparatus for refining lead, in combination, a vessel for holding molten lead containing crystals and a device for continuously moving crystals out of the lead while leaving the molten material behind.
9. In apparatus for refining lead, in combination, a vessel for holding molten lead containing crystals and a screw conveyor for moving crystals out of the lead while leaving the molten material behind.
10. A crystallizer-kettle unit for lead refining having in combination, a crystallizing trough feeding into a kettle and a device for moving crystals from the crystallizing trough into the kettle.
11. A crystallizer-kettle unit for lead refining having in combination, a crystallizing trough feeding into a kettle and a rotating screw conveyor for moving crystals from the crystallizing trough into the kettle.
12. A crystallizer-kettle unit for lead re-

fining having in combination, a crystallizing trough feeding into a kettle and a rotating screw conveyor, having holes pierced therein for allowing molten lead to drain from lead crystals, for moving crystals from the crystallizing trough into the kettle.

13. A crystallizer-kettle unit for lead refining having in combination, a crystallizing trough feeding into a kettle and a device for moving crystals from the crystallizing trough into the kettle, and a heater for melting crystals delivered to the kettle.

14. A crystallizer-kettle unit for lead refining having in combination, a crystallizing trough feeding into a kettle and a rotating screw conveyor for moving crystals from the crystallizing trough into the kettle, and a heater for melting crystals delivered to the kettle.

15. A crystallizer-kettle unit for lead refining having in combination, a crystallizing trough feeding into a kettle and a rotating screw, having holes pierced therein for allowing molten lead to drain from lead crystals, for moving crystals from the crystallizing trough into the kettle, the crystallizing trough and screw being set at an angle to the horizontal whereby the crystals are moved upwardly out of the solution on an incline and deposited in the kettle.

16. A crystallizer-kettle unit for lead refining having in combination, a crystallizing trough feeding into a kettle and a rotating screw conveyor, having holes pierced therein for allowing molten lead to drain from lead crystals, for moving crystals from the crystallizing trough into the kettle, the crystallizing trough and screw being set at an angle to the horizontal whereby the crystals are moved upwardly out of the solution on an incline and deposited in the kettle, a heater delivering products of combustion to said kettle for melting crystals deposited therein, and ducts positioned on the walls of said crystallizer above the level of the lead bath therein for conveying said products of combustion past said crystallizer to supply heat to the portions thereof situated above said bath.

In testimony whereof I have signed my name to this specification.

ARTHUR E. HALL.

120

125

130